

## UNITED STATES PATENT OFFICE.

FRANK A. FAHRENWALD, OF CLEVELAND HEIGHTS, OHIO.

## PROJECTILE.

No Drawing. Application filed December 15, 1919, Serial No. 845,082. Renewed June 20, 1924.

To all whom it may concern:

Be it known that I, FRANK A. FAHRENWALD, a citizen of the United States, residing at Cleveland Heights, in the county of 5 Cuyahoga and State of Ohio, have invented a certain new and useful Improvement in Projectiles, of which the following is a full, clear, and exact description.

This invention relates to projectiles, both 10 those which are employed in hand fire arms, as rifles, and those which are employed in larger fixed pieces such as heavy ordnance, and has for its object to improve the construction of the same so as to increase the 15 life of the barrels from which the same are fired. In all high velocity arms or ordnance it is necessary to use a jacket or driving band or bands to impart a rapid spinning motion to the projectile through engagement with the spiral ribs and grooves 20 formed on the interior of the bore. Lead is too soft and melts too easily, besides fouling the barrel interior very rapidly, especially when the same is made of iron or steel. 25 Lead is employed for the bullets of hand arms owing to its high specific gravity, but to prevent it from becoming melted by friction it is, in high velocity arms, encased in a jacket of harder and less fusible material. 30 In larger ordnance the projectile is usually of some kind of steel and is formed near its base with one or more external grooves which are filled with a suitable metal or alloy which shall engage the rifling and 35 serve the double function of setting the projectile in rotation and preventing the leakage of gas therewith.

Lead is inapplicable to this use for the 40 reasons above mentioned. Pure copper does not foul the bores, but is too soft for use in heavy ordnance, and when used for bullet jackets it becomes covered with a poisonous green coating by exposure to salt solutions and atmospheric conditions. In order to prevent this the expedient has been 45 tried of coating this copper jacket with an outside layer of tin, which serves that purpose successfully but offers the disadvantage of fouling the rifle bore more rapidly than any other one thing; with the possible exception of nickel. Pure soft iron (or a mild steel having a carbon content of less than two-tenths per cent) has been extensively 50 tried, but produces excessive barrel wear.

55 The object of my invention is the improvement of projectiles in respect to these

jackets, or bands in such wise that they shall neither foul nor erode the barrel, nor become corroded upon exposure, that they shall be soft enough to take the rifling and 60 also strong enough to set the projectile into rotation, and shall not be of high intrinsic value; while further objects and advantages of my invention will become apparent as this description proceeds. 65

I have discovered that the fouling effect of such a jacket or band upon the barrel is in proportion to its affinity for the metal of which the barrel is made, or in other words to the ease with which it would alloy 70 under ordinary conditions with the metal of the barrel, which alloying tendency is peculiarly stimulated under the conditions of high pressure and high temperature and close frictional contact. Thus nickel which 75 is one of the worst offenders in this regard is a metal which alloys with iron with particular ease. Tin likewise is easily combined with iron; while the high rate of wear 80 noticeable when iron guiding bands are used is apparently due to the same alloying but in this case the metal is abstracted from the bore rather than from the projectile.

It is therefore necessary to employ for this purpose some metal which alloys with 85 the barrel material only with difficulty if at all and I have discovered that in the case of an iron or steel barrel all the advantages sought by this invention can be obtained and all the disadvantages present in previous 90 attempts can be avoided by the use of certain alloys of aluminum or an aluminum-like metal.

Pure aluminum is for many purposes deficient in mechanical strength and hardness 95 and also has too low a melting point, but commercial aluminum, containing as it does up to two or three per cent of various hardening metals in the form of impurities, of which iron and copper are the chief, will 100 serve most purposes with great success. However, I prefer to employ the alloy of such metal with copper, and while it is perfectly possible to employ an alloy containing a large proportion of aluminum with a 105 small proportion of copper, I prefer to employ an alloy containing a comparatively large amount of copper and a small amount of aluminum or aluminum-like metal.

My preferred projectiles are made, particularly for high velocity arms and ordnance, with jackets or bands consisting of 110

2

copper alloyed with from about one per cent to about seven per cent of an aluminum-like metal (aluminum or magnesium or both). Even so small an amount of aluminum or magnesium as one per cent when alloyed with copper changes markedly the appearance of the metal, increases its hardness and resists its corrosion. Above about seven per cent of copper or magnesium the alloy 5 becomes too hard for most purposes. In case other hardening metals such as manganese, iron, nickel, or cobalt are present in any degree, it is necessary to decrease the amount of aluminum or magnesium, since 10 the heavy metals have a disproportionate effect upon the properties of hardness.

For a second composition falling within my invention but slightly less desirable, I employ aluminum from about 99% to about 20 93%, the balance being either pure copper or manganese, iron, nickel, cobalt, or some mixture thereof; this can be expressed as consisting of aluminum together with from about one to about eight per cent of one 25 or more hardening metals having atomic weight between about 55 and about 64 in the periodic table. Iron or nickel when present up to about three per cent, which is substantially the highest permissible limit 30 owing to their hardening effect do not seem to be able to exert any deleterious effect upon the barrel, since the presence in the alloy of less than about 5% of the barrel substance appears to be too great a dilution 35 to lead to combination.

As a third modification I may employ from about 99% to about 92% of aluminum with the balance of magnesium, which is 40 satisfactory as regards its hardness and strength, but is not as well considered because of its very low specific gravity. For the same reason all the alloys containing

the larger amounts of aluminum are less desirable than those containing the small amounts. It will be understood, however, 45 that magnesium can be used in connection with the aluminum in all cases, the total amount of magnesium being in all instances maintained at less than about ten per cent 50 of the whole alloy.

It will be understood that the alloys containing the larger proportions of aluminum, in addition to being unduly light in weight will be too fusible for some purposes where extremely high velocities are used, since all 55 these high aluminum alloys are more fusible than aluminum itself; however, the alloy with copper, by reason of its smoothness and well known lubricating qualities offsets to some extent this low melting point. The 60 low aluminum, high copper alloy has no drawbacks whatever and further possesses an inherent smoothing and lubricating quality which is very beneficial to the arm.

Having thus described my invention, what I claim is:—

1. A projectile for firearms having a surrounding band or jacket made of an alloy of aluminum together with from about 1% to about 8% of a hardening metal having 70 an atomic weight between 55 and 64.
2. A projectile for firearms having a surrounding band or jacket made of an alloy of aluminum and between 1% and 8% of copper. 75
3. A jacket or driving band made of an alloy containing aluminum with about 1% to about 8% of one or more hardening metals having an atomic weight between 55 and 64. 80

In testimony whereof, I hereunto affix my signature.

FRANK A. FAHRENWALD.